

Feb. 16, 1926.

1,573,708

W. F. HOERLE

MANUFACTURE OF GOLF CLUB SHAFTS

Original Filed Nov. 18, 1924

Fig. 1.



Fig. 2.



Fig. 3.



Fig. 4.



Fig. 5.



Fig. 6.



Fig. 7.



Inventor

William F. Hoerle  
By his Attorney  
R. W. Flynn.

Patented Feb. 16, 1926.

1,573,708

# UNITED STATES PATENT OFFICE.

WILLIAM FERDINAND HOERLE, OF TORRINGTON, CONNECTICUT, ASSIGNOR TO UNION HARDWARE COMPANY, OF TORRINGTON, CONNECTICUT, A CORPORATION OF CONNECTICUT.

## MANUFACTURE OF GOLF-CLUB SHAFTS.

Original application filed November 18, 1924, Serial No. 750,516. Divided and this application filed July 2, 1925. Serial No. 41,229.

To all whom it may concern:

Be it known that I, WILLIAM F. HOERLE, a citizen of the United States of America, residing at Torrington, county of Litchfield, 5 State of Connecticut, have invented a new and useful Manufacture of Golf-Club Shafts, of which the following is a specification.

My invention relates to the art of making 10 handles or shafts for golf clubs and this application is a division from application #750,516, filed November 18, 1924.

The ordinary wooden shaft is, of course, 15 quite flexible and has desirable torsional characteristics which make the club lively, but it is very fragile, uncertain in quality and considerably affected by moisture. It has heretofore been proposed to make such devices of steel. Some of these devices, however, have been very heavy and non-torsionable and others very fragile. Shafts have 20 been made of steel strips formed into tubes but these are difficult to make uniformly and are likely to split open. So far as I know 25 no one has heretofore been able to produce commercially an integral or seamless tubular golf club shaft sufficiently well balanced, light and pliable to be useful and yet sufficiently strong to stand the severe stresses to 30 which such a shaft is subjected.

The main object of my invention is to 35 provide a method of making a light but strong, smooth and durable metallic shaft which will look and act very much like a first-class wooden shaft and yet not have the 40 objectionable characteristics of wood.

I have also sought to provide a method of making shafts commercially according to standard specifications and at a low cost.

45 I have found it possible to make a satisfactory shaft from an ordinary cylindrical low carbon seamless steel tube by forming, shaping or drawing it, then carbonizing the tube and heat treating and finishing it.

45 Figure 1 is a side view of a golf club of standard form having a shaft made according to my invention.

Fig. 2 is a side view of a tubular blank from which a shaft is made.

50 Fig. 3 is a side view of a finished shaft.

Figs. 4 and 5 are transverse sectional views of the shaft on an enlarged scale taken re-

spectively at the upper and lower ends of the shaft.

Figs. 6 and 7 are enlarged detail sectional views showing different ways of fastening a shaft in a head.

According to the preferred method of manufacture I use a blank 7 of seamless tubing of low carbon steel having say from 60 about 10 to 40 points of carbon that is from about .1 to .4 of one percentum of carbon. The outside diameter of the blank tube may be about  $\frac{5}{8}$  of an inch which may be the diameter of the handle end of the shaft. 65 The gauge of the metal is preferably from .015" to .018", although it may be slightly more or less. About .016" is quite desirable for a driver shaft.

This blank is formed, rolled or swaged so 70 as to reduce the diameter to the desired size at the head end. For instance an ordinary golf club shaft would be something over 3 feet long and approximately  $\frac{1}{16}$  of an inch in diameter at the smallest point in the neck. 75 8. The reducing process should preferably elongate the tube and leave the wall thicker in the small neck than at the larger handle end. An elongation of ten per cent is usual. That is, from say 36" to 40". The torsibility of the tube gradually increases as the section is taken nearer the small end. This 80 also makes the tube more flexible in the neck. A satisfactory thickness of the wall at the neck would be .019", although it may be a 85 little thicker or a little thinner than this.

After the tube has been worked to the desired shape and size, it is carbonized in a suitable manner, for instance in a gas fired tube or in a charcoal or coke furnace or 90 electrically. This is done, preferably, at a comparatively low temperature, say 1450° F. so as not to injure the steel. This carbonizing is continued until the carbon content of the steel is increased to a suitable amount 95 for the purpose required, say from six tenths to one percentum. The carbon content can be increased even somewhat above one percent by careful treatment but I do not consider it necessary to go above .75 to .80 and 100 in some cases a tube with even less than .75 percentum of carbon can be heat treated and hardened.

The tube is then heat treated and drawn

to the desired temper. It may then be provided with a suitable noncorrosive finish. Such a shaft should weigh from about five to six ounces.

5 The length of course is a matter of accommodation to the individual. The weight will necessarily vary with the length. The weight and stiffness of some clubs is of course less critical than others. For instance, a putter 10 shaft does not need to be as flexible or torsible as a driver.

A low carbon steel tube is not only less expensive than a high carbon tube but it is much cheaper and easier to work without 15 injury to the metal. The rolling or swaging is preferably done cold and not only compacts the metal but draws out the fibre in the direction of the length of the shaft particularly in the smaller part so as to utilize 20 the strength of the metal to its maximum extent. The working of the tube may be effected to produce a taper effect if desired. The carbonizing and heat treating processes release the internal stresses developed by the 25 prior working process and make the steel susceptible of hardening and tempering a higher degree than would be possible with a low carbon steel. Carbonizing of a low carbon steel when properly done produces a 30 condition where there is more carbon in the metal near the surface than there is inside. Consequently when hardened and tempered we have a hard exterior or skin and a softer interior and the tube is resilient and yet 35 tougher and stronger than is possible to get in a tube made from a so called high carbon steel.

The upper or handle end 9 of the tube may be left of uniform diameter if desired 40 and provided with any suitable form of grip 10.

The shaft may be used with any style head. In Figure 1 I have shown a putter 45 or iron provided with a socket 11. To fit such a socket I may provide the lower end 50 of the shaft with a tapered enlargement 12 integral with the shaft and adapted to be fitted and held in the socket of the head in the same manner that a wooden shaft is held. 55 It should be understood, of course, however, that the lower end may be inserted and held in any form of wooden head in substantially the same manner that a wooden shaft is held.

55 In some cases it may be desirable to reinforce the tube adjacent the head by means of a ferrule or plug such as 13 in Fig. 6. The curved end adjacent the entrance to the socket in the head 14 permits slight bending of the shaft and yet reinforces it 60 at this point where the stress is very great.

In case the socket 15 of the head is larger than the end of the shaft I may employ a 65 filler ferrule 16. An inner plug 17 may be used to spread the end of the shaft in the

socket and prevent the metal from buckling.

A pin 18 may be used to hold the parts together. A filler and plug would both serve to reinforce the tube at this point.

Such a shaft not only has the requisite 70 strength to resist crushing and bending but it has torsional and flexible characteristics closely resembling those of a wooden shaft of high grade. Since the shaft is drawn, rolled or swaged from a seamless tube, there 75 are no joints liable to open when the club is used and subjected to the severe strains of ordinary play. By this process it is possible to make shafts commercially in quantity production and with such standard characteristics as may be desired as to cost, 80 weight, flexibility and torsibility.

I claim:

1. The process of forming a golf club shaft which comprises working and tapering a seamless steel tube having a carbon content of .10 to .40 percentum, carbonizing the tapered tube to increase the carbon content to about six tenths to one percentum, then heat treating, hardening and tempering 85 said tube.

2. The process of forming a tubular golf club shaft which comprises rolling and elongating the fibre of a thin walled low carbon seamless steel tube and reducing the 95 diameter at one end, then heating and carbonizing said tube to materially increase the carbon content throughout its thickness and then heat treating, hardening and tempering 100 said tube.

3. The process of forming a golf club shaft which comprises tapering a very thin walled low carbon seamless steel tube, carbonizing the tapered tube to substantially increase the carbon content throughout the 105 entire thickness of the wall of the tube, then heat treating and hardening and tempering said tube.

4. The process of forming a tubular golf club shaft which comprises elongating and 110 reducing a seamless drawn tube so as to increase the thickness of the metal and reduce the diameter at its lower end, then heating and carbonizing said tube to release internal stresses and increase the carbon content, and then hardening and tempering 115 said tube.

5. The process of forming a tubular golf club shaft which comprises elongating a low carbon seamless tube about ten percentum 120 and increasing the thickness of the metal at its lower end less than one hundred percentum, and decreasing the diameter of the tube at its lower end, then heating and carbonizing said tube to increase the carbon content to above .6 of a percentum, and then heat treating, hardening and tempering said tube.

6. The process of forming a golf club shaft which comprises working a seamless 125

steel tube having a carbon content of .10 to .40 percentum, reducing its diameter at one end, carbonizing the tube to increase the carbon content to about six tenths to one 5 percentum, then heat treating, hardening and tempering said tube.

7. The process of forming a tubular golf club shaft which comprises elongating a seamless drawn tube so as to increase the 10 thickness of the metal at its smaller end, then heating and carbonizing said tube to release internal stresses and increase the carbon content, and then hardening and tempering said tube.

15 8. The process of forming a flexible and torsionable shaft for a golf club which comprises working a thin walled low carbon seamless steel tube so as to elongate the

tube and reduce the diameter at one end, then heating and carbonizing the tube so 20 as to add at least five tenths of one percentum of carbon to the metal and then heat treating, hardening and tempering the carbonized tube.

9. The process of forming a flexible and 25 torsionable shaft for a golf club which comprises working a thin walled low carbon steel tube at atmospheric temperature to elongate it and reduce the diameter at one end, then carbonizing the tube at a temperature of approximately 1450° F. to materially increase the carbon content, then heat treating, hardening and tempering the carbonized tube. 30

WILLIAM FERDINAND HOERLE.